

2,848,420

## NONTARNISHING DETERGENT COMPOSITIONS

Charles H. Schramm, Hillsdale, N. J., assignor to Lever Brothers Company, New York, N. Y., a corporation of Maine

No Drawing. Application July 12, 1954  
Serial No. 442,895

23 Claims. (Cl. 252—137)

This invention relates to cleaning compositions containing tarnish inhibitors and more particularly to polyphosphate and synthetic detergent compositions containing guanamine compounds as tarnish inhibitors.

Compositions containing polyphosphates and/or synthetic detergents are now widely used for detergent and other purposes. Aqueous solutions of polyphosphates and some synthetic detergents tend when at certain pH values to tarnish copper, and nickel and copper alloys such as German silver (a nickel-zinc-copper alloy) to a variety of shades from yellow to bluish black, especially if the solutions are at elevated temperatures and are allowed to remain in contact with the metal for several minutes. Since German silver is frequently used for household articles commonly washed in polyphosphate-built detergent compositions, it is evident that this is a serious problem.

In accordance with the instant invention polyphosphate and detergent compositions are provided containing a tarnish inhibitor which compositions will not tarnish copper, and nickel and copper alloys such as German silver. The tarnish inhibitor of the invention is a substituted guanamine (2,4-diamino-s-triazine) which is described by the following formula:



where at least one R is a hydrocarbon or heterocyclic radical and can be selected from the group consisting of aliphatic, aryl, mixed alkylene aryl, mixed phenylene heterocyclic and mixed alkylene heterocyclic hydrocarbon radicals, and the other R radicals can be hydrogen or any of the radicals selected from the above-mentioned group.

When R is an aliphatic hydrocarbon group it can have either a straight or branched chain, and can be saturated or unsaturated.

The number of carbon atoms in the R groups is important. Formoguanamine is not effective. Good tarnish-inhibiting properties appear when at least one of R<sub>1</sub>, R<sub>2</sub>, R<sub>3</sub>, R<sub>4</sub> or R<sub>5</sub> is a radical having three carbon atoms and the remaining R groups are hydrogen, but relatively large amounts of such guanamines may be necessary for complete protection. Tarnish-inhibiting ability materially improves as the R groups increase further in molecular weight, and lesser amounts of guanamine can be used. Optimum tarnish-inhibiting properties are displayed by compounds in which the sum of the R groups is from seven to seventeen carbon atoms, especially compounds in which at least one R has from seven to seventeen carbon atoms, and in such compounds the number of carbon atoms in the remaining R groups is not critical, although the lower alkyl groups,

i. e., those having from one to about five carbon atoms, and hydrogen are preferred.

Typical R radicals are straight and branched chain methyl, ethyl, propyl, heptyl, octyl, nonyl, butyl, hexyl, decyl, undecyl, dodecyl, tridecyl, tetradecyl, pentadecyl, decenyl, heptylenyl, hexadecyl, heptadecyl, decynyl, dodeceny, octadecenyl, octadecadienyl, dodecynyl, the mixed alkyl radicals derived from fatty oils such as palm oil, rapeseed oil, tall oil, linseed oil, etc., phenyl, benzyl, phenyl guanamyl, decylene guanamyl and octylene guanamyl. These can be taken in any combinations meeting the above requirements.

The following are some typical guanamines in accordance with the invention:





Others are given in the examples.

These guanamines are in many instances known compounds and are readily prepared by reaction of a substituted biguanide (guanyl guanidine) and the corresponding nitrile, acid or ester (1) using a mononitrile or monocarboxylic acid or ester in a 1:1 molar ratio if one guanamine radical is to be present and (2) using a dinitrile or dicarboxylic acid or ester in a 2:1 molar ratio if two guanamine radicals are to be present. The reaction proceeds in accordance with the following equations:



The mixture of the nitrile, acid or ester and biguanide is heated at an elevated temperature, say 180° C., for several hours. Temperatures from 120 to 250° C. have been found satisfactory.

The crude mixture which is obtained as a result of this reaction can be used without further purification and consists mainly of the substituted guanamide and, in the case of acid or ester reactants, of the amide of the acid or ester starting material in approximately equal amounts. The guanamine has been isolated and shown to be the principal antitarnishing constituent of the mixture.

The guanamines in accordance with the invention are nontoxic, sparingly water-soluble substances, but suffi-

ciently water-soluble to permit their incorporation in polyphosphate and synthetic detergent solutions in the amounts required to impart tarnish inhibition thereto.

An amount of the guanamine would be added to the 5 polyphosphate and/or synthetic detergent composition sufficient to give tarnish inhibition when the composition is used in its normal way. Usually about 0.1% of the 10 guanamine gives adequate tarnish inhibition, but larger amounts can be used if desired. From 0.1 to 5% is 15 effective under nearly all conditions and therefore is preferred. The maximum amount of guanamine is not critical but more than is necessary to give the desired effect usually would not be used, and of course an amount 20 in excess of that soluble in the solution would not be used. It will be understood that the amount required will depend in part upon the tarnish-inhibiting properties of the particular guanamine in question, upon the tendency 25 of the polyphosphate and/or synthetic detergent with which it is used to tarnish copper and nickel alloys and copper alloys, and upon the amounts of polyphosphate and synthetic detergent present.

The guanamines of the invention are effective as tarnish inhibitors in both hard and soft water.

The tarnish inhibitors of the invention are effective 25 with water-soluble polyphosphates as a class at pH values where such polyphosphates tend to tarnish German silver (usually pH 6 or above) and particularly those polyphosphates identified by the following general formula from which it is seen that both the acids and their various 30 salts are contemplated:

$$[(\text{M}_1\text{M}_2\text{M}_3\text{PO}_4)_a \text{ minus } b(\text{MOM})]_x$$

where:

35  $\text{M}_1, \text{M}_2$  and  $\text{M}_3$  are hydrogen or an alkali metal, such as sodium, potassium and ammonium, and can be the same or different, and  $\text{M}$  is  $\text{M}_1$  and/or  $\text{M}_2$  and/or  $\text{M}_3$ .  $a$  is an integer of 1 or more, usually 1 to 4, 40  $b$  is an integer of 1 or more, usually 1 or 2,  $x$  is an integer of 1 or more, usually 1 to 6.

In the case where  $a$  is 2,  $b$  is 1 and  $x$  is 1, the compound is 45 a pyrophosphate. When  $a$  is 1,  $b$  is 1 and  $x$  is 1, the compound is a metaphosphate. Others will be evident to those skilled in the art.

The upper limit of  $a$ ,  $b$  and  $x$  is not critical, but will be determined by the increasingly lower water-solubility as molecular weight increases. The sodium polyphosphates are preferred.

As the general formula shows, both the normal and acid salts of the phosphates are within the scope of the invention.

55 Among the polyphosphoric acids and their alkali metal salts coming within the invention are the polymetaphosphoric acids  $(\text{HPO}_3)_x$ , ( $a$  is 1,  $b$  is 1,  $x$  is more than 1), pyrophosphoric acid  $\text{H}_4\text{P}_2\text{O}_7$  ( $a$  is 2,  $b$  is 1,  $x$  is 1), triphosphoric acid  $\text{H}_5\text{P}_3\text{O}_{10}$  ( $a$  is 3,  $b$  is 2,  $x$  is 1), and tetraphosphoric acid  $\text{H}_6\text{P}_4\text{O}_{13}$  ( $a$  is 4,  $b$  is 3,  $x$  is 1).  $\text{Na}_5\text{P}_3\text{O}_{10}$ ,  $\text{K}_4\text{P}_2\text{O}_7$ ,  $\text{Na}_4\text{P}_2\text{O}_7$ ,  $\text{Na}_2\text{H}_2\text{P}_2\text{O}_7$ ,  $\text{Na}_4\text{P}_4\text{O}_{13}$ , Sodium Polyphos (Na<sub>12</sub>P<sub>10</sub>O<sub>31</sub>—Blockson), K<sub>4</sub>(PO<sub>3</sub>)<sub>4</sub>·2H<sub>2</sub>O, Pascal's salt, sodium dimetaphosphate, sodium trimetaphosphate (Knorre's salt), sodium tetrametaphosphate and sodium hexametaphosphate (Graham's salt) are examples.

65 The guanamine tarnish inhibitors can be incorporated in compositions containing polyphosphates, and in compositions containing synthetic detergents, and are effective to reduce tarnish due to polyphosphate or detergent in each of these types of compositions. They are particularly useful in synthetic detergent compositions which contain one or more polyphosphates as builders and one or more synthetic detergents, i. e., anionic detergents, cationic detergents, nonionic detergents, and mixtures 70 thereof. In many instances they display an enhanced 75

tarnish-inhibiting action in the presence of both polyphosphate and detergent.

The polyphosphate-built detergent compositions should contain conventional proportions of active detergent, usually within the range between 5 to 40%, polyphosphate in any amount, usually between 5 to 50%, based on the total composition, and the residue builders and inert materials.

The guanamines are useful with a wide variety of anionic, cationic and nonionic synthetic detergents, with and without polyphosphates.

The alkyl aryl sulfonates are a class of detergents well known in the art under this name. One example thereof are the sulfonated phenylpolypropylene alkanes, characterized by the branched chain structure of polypropylene and a tertiary alkyl carbon at the benzene ring, and having the following general structure:



where M is hydrogen, an alkali metal or an organic amine cation, and R<sub>1</sub> and R<sub>2</sub> are alkyls, of the type formula C<sub>n</sub>H<sub>2n+1</sub>, and at least one R is a polypropylene group, the whole alkyl group containing preferably twelve to fifteen carbon atoms. These are known compounds, whose preparation and properties are set forth in U. S. Patent No. 2,477,383 to Lewis, issued July 26, 1949; they are available in commerce under the trade names "Oronite," "Ultrawet" and "Neolene."

Another class of useful detergents are the amidoalkane sulfonates which are characterized by the following structure:



where A is hydrogen or an alkali metal, i. e., ammonium, sodium, or potassium, n is a small whole number from one to about five, preferably two or three, R' is hydrogen, or an alkyl, aryl, or cycloaliphatic group, such as methyl, and R is an alkyl or alkylene radical, such as myristyl, palmityl, oleyl and stearyl. Sodium palmitic tauride, sodium palmitic methyl tauride, sodium myristic methyl tauride, sodium palmitic-stearic methyl tauride and sodium palmitic methyl amidopropane sulfonate have been found to be particularly suitable for use in the compositions of the invention.

These compounds are prepared by interacting the corresponding aliphatic acid anhydride or halide with an organic aliphatic aminosulfonic acid, such as taurine



and the various N-substituted taurines, such as N-methyl taurine, or aminopropane sulfonic acid, NH<sub>2</sub>(CH<sub>2</sub>)<sub>3</sub>SO<sub>3</sub>H.

The invention is also applicable to other water-soluble alkyl aromatic sulfonic acids, such as those prepared by alkylating benzene or naphthalene with a kerosene fraction followed by sulfonation to aliphatic sulfonic acids, esters of sulfuric acid with aliphatic alcohols of ten to eighteen carbon atoms, particularly those derived by the reduction of coconut oil, palm oil and like long-chain fatty acids, sulfonated castor oil, esters and ethers of isethionic acid, long-chain fatty acid esters and long-chain alkyl ethers of 2,3-dihydroxy propane sulfonic acid and sulfuric acid esters of monoglycerides and glycerol monoethers. The salts of these acids are ordinarily employed.

The tarnish-inhibitors are also useful with nonionic detergents, such as, for example, alkyl oxyether and ester

and thioether and ester detergents having the following general formula:



where R is a straight or branched chain saturated or unsaturated hydrocarbon group having from eight to eighteen carbon atoms or an aralkyl group having a straight or branched saturated or unsaturated hydrocarbon group of from eight to eighteen carbon atoms attached to the aryl nucleus, and attached to A through the aryl nucleus, A is selected from the group consisting of ethereal oxygen and sulfur, carboxylic ester and thiocarboxylic ester groups and x is a number from eight to twenty. R can for example be a straight or branched chain octyl, nonyl, decyl, lauryl, myristyl, cetyl or stearyl group, or an alkyl aryl group such as octylbenzene, nonylbenzene, decylbenzene, stearylbenzene, etc.

The sulfated ethoxynated derivatives of the above also are useful anionic detergents:



where M is hydrogen or an alkali metal or organic amine cation and x, A and R are as above.

When R is alkyl it will be evident that the detergent can be regarded as derived from an alcohol, mercaptan, oxy or thio fatty acid of high molecular weight, by condensation with ethylene oxide. Typical of this type of alkyl ether are the condensation products of oleyl or dodecyl alcohol or mercaptan with from eight to seventeen moles of ethylene oxide, such as "Emulfor ON," "Nonic 218" and "Sterox SE" and "SK." Typical alkyl esters are "G1226" and "Renex" (polyoxyethylene ester of tall oil acids), "Sterox CD" and "Neutronyx 330" and "331" (higher fatty acid esters of polyethylene glycol). When R is aralkyl, the detergent can be derived from an alkyl phenol or thiophenol.

The ethoxynated alkyl phenols and thiophenols have the following general formula:



where R is a straight or branched saturated or unsaturated hydrocarbon group having at least eight carbon atoms up to approximately eighteen carbon atoms, A is oxygen or sulfur and x is a number from eight to twenty. R can, for example, be a straight or branched chain octyl, nonyl, decyl, lauryl, cetyl, myristyl or stearyl group. Typical are the condensation products of octyl and nonyl phenol and thiophenol with from eight to seventeen moles of ethylene oxide, available commercially under the trade names "NIW," "Antarox A-400," "Igepal CA" and "CO," "Triton X-100," "Neutronyx 600" and "Tergitol NFX."

The detergent composition can contain supplemental builders including alkali metal and alkaline earth metal sulfates, chlorides, silicates, borates, carbonates, metaphosphates, and orthophosphates, such as sodium silicate, magnesium sulfate, sodium tetraborate, sodium carbonate, sodium sulfate, trisodium phosphate, potassium carbonate, disodium orthophosphate, sodium metaphosphate, calcium sulfate, calcium chloride, sodium chloride, sodium borate and potassium metaphosphate. The builder should but need not be water-soluble.

In addition to or instead of the above-mentioned supplemental inorganic salts, organic materials such as starch, polyethylene glycols, polyvinyl alcohols and salts of carboxymethylcellulose can be used as builders. It has been found that between about 0.1 and 1% of an alkali metal carboxymethylcellulose increases detergency and sudsing.

The builder mixture is so chosen among alkaline, neutral and acidic salts that the composition obtained in an aqueous 0.14% washing solution has a pH of 7 or above. Preferably, its pH lies within the range from 7 to about 10 since solutions which are more alkaline may be irritating to the skin and tend to weaken some fabrics, particularly woolens. In general, the alkali metal carbonates are preferred agents for bringing the pH of the solution to a high alkaline value within the preferred range.

The detergent composition is prepared by conventional methods, as by blending the ingredients thereof in an aqueous solution or slurry and then drying the resulting mixture in a spray or drum dryer at elevated temperatures.

The tarnish inhibitor may be added to the polyphosphate or detergent composition at any stage of its manufacture, to the finished polyphosphate or detergent composition, or to the polyphosphate or detergent solution.

The guanamines employed in the following examples were prepared by heating mixtures of biguanide and the corresponding nitrile at 150-200° C. for about two to four hours. 1:1 molar ratios were taken of biguanide and the nitrile. The crude product was used unless otherwise indicated.

In the examples the tarnishing action of the compositions was evaluated by this test:

Five grams (dry solids basis) of the composition to be tested is dissolved in one quart of distilled water and 300 ml. of the test solution placed in a suitable container and brought to 160° F. A strip of German silver metal is polished with a metal polish, washed and dried, placed in the solution and the solution held at 160 to 170° F.

for one-half hour. The effectiveness of the inhibitor is rated as follows:

Excellent=no more than slight or barely noticeable cast, uniform or spotted.

Fair=very slight to considerable attack.

Tarn=severely tarnished, same as when inhibitor is absent.

#### EXAMPLES 1 TO 4

10 Detergent compositions were prepared having the following formulation:

|                                                                | Percent |
|----------------------------------------------------------------|---------|
| Sodium Oronite (active) (sodium phenylpolypropylene sulfonate) | 18.0    |
| 15 Tetrasodium pyrophosphate                                   | 30.0    |
| Sodium tripolyphosphate                                        | 15.0    |
| Sodium carboxymethylcellulose                                  | 0.5     |
| Sodium silicate                                                | 6.0     |
| 20 Sodium carbonate                                            | 3.0     |
| Sodium sulfate and misc                                        | 20.5    |
| Water                                                          | 7.0     |
|                                                                | 100.0   |

25 Guanamine <sup>1</sup> 0.02 to 5

<sup>1</sup> 0.044 to 11.1% based on the weight of the polyphosphates.

To solutions of these compositions were added the alkyl guanamines listed in the table below in the amount indicated and for comparison purposes a control was prepared which did not contain any tarnish inhibitor. The solutions then were tested for tarnish inhibition in accordance with the above-described test with the following results:

Table I

| Example No.  | Inhibitor                                                                                                         | Percent Inhibitor |       |       |       |
|--------------|-------------------------------------------------------------------------------------------------------------------|-------------------|-------|-------|-------|
|              |                                                                                                                   | 0.02%             | 1.0%  | 2.0%  | 5.0%  |
| Control..... | None                                                                                                              | Tarn.             | Tarn. | Tarn. | Tarn. |
| 1            | <br>Formoguanamine            | Tarn.             | Tarn. | Tarn. | Tarn. |
| 2            | <br>4-N-Phenyl Formoguanamine | Tarn.             | Exc.  | Exc.  | Exc.  |
| 3            | <br>Stearoguanamine           | Tarn.             | Exc.  | Exc.  | Fair. |
| 4            | <br>Lauroguanamine            | Tarn.             | Exc.  | Exc.  | Exc.  |

Exc.=excellent.

It is evident from the above results that formoguanamine, a guanamine without an R substituent, is not effective as a tarnish inhibitor. A compound in which one of R<sub>1</sub>, R<sub>2</sub>, R<sub>3</sub>, R<sub>4</sub> or R<sub>5</sub> is an alkyl radical or an aryl radical and the remaining R's hydrogen is effective, however, as evidenced by 4-N-phenyl formoguanamine, a compound where R<sub>4</sub> is phenyl, and stearoguanamine and lauroguanamine, compounds where R<sub>1</sub> is a higher alkyl group.

The compositions also were evaluated for their sudsing properties. This was done using the Terg-O-Tometer employing the following procedure: 2.64 g. of the detergent composition without the tarnish inhibitor was weighed into a 100 ml. beaker and the appropriate amount of the tarnish inhibitor to be tested was added. Fifty ml. of 50 p. p. m. water was then added and the solids brought into solution with the aid of heat. The solution was diluted to 1,000 ml. with 50 p. p. m. water, brought to 120° F. and placed in the cup of a standard Terg-O-Tometer. 0.75 g. vacuum cleaner dust soil was then added, followed by twelve 4½" x 6" pieces of desized cotton sheeting. The paddles of the Terg-O-Tometer were operated for ten minutes at the rate of eighty-six complete oscillations per minute, while maintaining the temperature of the solutions at 120° F. After the ten minute period the quantity of suds was visually estimated and graded according to the following scheme:

Grade 0=no suds  
 Grade 1=trace of suds  
 Grade 2=trace to ½ coverage of surface  
 Grade 3=½ to ¼ coverage of surface  
 Grade 4=¼ to ¾ coverage of surface  
 Grade 5=¾ to ½ coverage of surface  
 Grade 6=½ to ¾ coverage of surface  
 Grade 7=¾ to full coverage of surface

The following results were obtained:

Table II

| Example No.  | Inhibitor                     | Percent Inhibitor |    |    |
|--------------|-------------------------------|-------------------|----|----|
|              |                               | 1%                | 2% | 5% |
| Control----- | No Guanamine:                 | 1                 | 1  | 1  |
| 1            | Formoguanamine<br>            | 1                 | 1  | 1  |
| 2            | 4-N-Phenyl Formoguanamine<br> | 1                 | 1  | 1  |
| 3            | Stearoguanamine<br>           | 1                 | 0  | 0  |
| 4            | Lauroguanamine<br>            | 1                 | 5  | 6  |

The above results show that lauroguanamine has excellent suds-boosting properties. These suds-boosting properties are not displayed by the other compounds tested, showing that compounds having an R<sub>1</sub> group of approximately twelve carbon atoms are unique in this respect. Similar suds-boosting properties would be expected from compounds having R<sub>1</sub> alkyl radicals of from ten to fourteen carbon atoms.

Compositions containing tarnish inhibitors of the invention do not tarnish copper, nickel-copper-zinc alloys such as German silver, coinage nickel or brass, which normally tarnish when exposed to aqueous solutions containing polyphosphates and/or synthetic detergents. It is not possible at this time to explain why the compounds of the invention are effective tarnish inhibitors.

Obviously, many modifications and variations may be made in the invention herein set forth without departing from the spirit and scope thereof, and only such limitations should be imposed as are indicated in the appended claims.

All parts and percentages in the specification and claims are by weight. Proportions of guanamine are based on the weight of the tarnish-producing substance, i. e., polyphosphate and/or detergent, unless otherwise stated. In the examples, for ease of preparation, the weights of guanamine are given as based on the dry weight of the total composition.

The nomenclature employed in this application and in the claims for the guanamines conforms with that used in the published literature. See U. S. Patent No. 2,459,710, for example. The guanamines are named in accordance with the acid from which they are prepared. The following table will clarify the relation between the R radicals in the general formulae in column 1, lines 39-45 and in the claims with the names of the guanamines as named elsewhere in the specification and claims:

| From Acid: | R Radical    | Guanamine  |
|------------|--------------|------------|
| 40         | formic       | hydrogen   |
|            | butyric      | propyl     |
|            | caprylic     | heptyl     |
|            | lauric       | heptadecyl |
|            | stearic      | heptadecyl |
|            | benzoic      | phenyl     |
|            | terephthalic | phenylene  |
| 45         | oxalic       | guanamyl   |
|            | succinic     | ethylene   |
|            | sebacic      | octylene   |

I claim:

1. A detergent composition consisting essentially of a water-soluble substance selected from the group consisting of polyphosphates and synthetic organic nonsoap anionic and nonionic detergents which in aqueous solution tarnishes copper and copper and nickel alloys and a tarnish inhibitor in an amount to lessen the tarnishing action of the substance and having the general formula:



where at least one R is an organic radical selected from the group consisting of hydrocarbon and guanamine radicals having at least three carbon atoms, and the remaining R radicals are selected from the group consisting of hydrogen, hydrocarbon, and guanamine radicals.

2. A detergent composition in accordance with claim 1 in which at least one R radical has from seven to seventeen carbon atoms.

3. A detergent composition in accordance with claim 1 which the tarnish inhibitor is lauroguanamine.

4. A detergent composition in accordance with claim 1 in which the tarnish inhibitor is capryloguanamine.

5. A detergent composition in accordance with claim 1 in which the tarnish inhibitor is stearoguanamine.

6. A detergent composition in accordance with claim 1 in which  $R_1$  is the mixed alkyl radicals derived from a naturally-occurring fatty oil.

7. A detergent composition in accordance with claim 1 in which  $R_1$  is a mixed alkylene aryl radical.

8. A detergent composition in accordance with claim 1 in which  $R_1$  is a mixed alkylene guanamine radical.

9. A detergent composition in accordance with claim 1 in which  $R_1$  is a mixed phenylene guanamine radical.

10. A detergent composition in accordance with claim 1 in which  $R_1$  is phenyl.

11. A detergent composition in accordance with claim 1 in which  $R_4$  is phenyl.

12. A detergent composition in accordance with claim 6 in which the fatty oil is palm oil.

13. A detergent composition in accordance with claim 6 in which the fatty oil is rapeseed oil.

14. A detergent composition in accordance with claim 6 in which  $R_1$  is the mixed alkyl radicals derived from tall oil.

15. A detergent composition in accordance with claim 7 in which the mixed alkylene aryl radical is benzyl.

16. A detergent composition consisting essentially of a water-soluble polyphosphate which in aqueous solution tarnishes copper and copper and nickel alloys and a tarnish inhibitor in an amount to lessen the tarnishing action of the polyphosphate and having the general formula:



where at least one R is an organic radical selected from the group consisting of hydrocarbon and guanamine radicals having at least three carbon atoms, and the remaining R radicals are selected from the group consisting of hydrogen, hydrocarbon, and guanamine radicals.

17. A detergent composition in accordance with claim 16 in which the amount of tarnish inhibitor is within the range from 0.5 to 5% by weight of the polyphosphate.

18. A detergent composition in accordance with claim 5 in which the polyphosphate is a tripolyphosphate.

19. A detergent composition in accordance with claim 16 in which the polyphosphate is a pyrophosphate.

20. A detergent composition in accordance with claim 16 in which the polyphosphate is a polymetaphosphate.

21. A detergent composition consisting essentially of a water-soluble synthetic organic nonsoap detergent selected from the group consisting of anionic and nonionic detergents which in aqueous solution tarnishes copper and copper and nickel alloys and a tarnish inhibitor in an amount to lessen the tarnishing action of the detergent and having the general formula:



25 where at least one R is an organic radical selected from the group consisting of hydrocarbon and guanamine radicals having at least three carbon atoms, and the remaining R radicals are selected from the group consisting of hydrogen, hydrocarbon and guanamine radicals.

22. A detergent composition in accordance with claim 30 21 in which the detergent is a phenylpolypropylene sulfonate.

23. A detergent composition in accordance with claim 21 in which the detergent is a condensation product of an alkylene oxide and an organic compound reactive therewith, selected from the group consisting of higher fatty carboxylic and thio carboxylic acids and higher fatty alcohols and mercaptans.

References Cited in the file of this patent

UNITED STATES PATENTS

2,618,603 Schaeffer \_\_\_\_\_ Nov. 18, 1952  
2,618,605 Schaeffer \_\_\_\_\_ Nov. 18, 1952

UNITED STATES PATENT OFFICE  
Certificate of Correction

Patent No. 2,848,420

Charles H. Schramm

August 19, 1958

It is hereby certified that error appears in the printed specification of the above numbered patent requiring correction and that the said Letters Patent should read as corrected below.

Column 8, Table I, second column thereof, opposite Example No. 3, the formula should appear as shown below instead of as in the patent—



column 10, line 72, after the claim reference numeral "1" insert—in—  
Signed and sealed this 28th day of October 1958.

[SEAL]

Attest:

KARL H. AXLINE,  
*Attesting Officer.*

ROBERT C. WATSON,  
*Commissioner of Patents.*